

Feb. 24, 1925.

1,527,305

T. W. S. HUTCHINS

ELECTRODEPOSITION OF METALS

Filed Feb. 5, 1923



Inventor:  
T. W. S. Hutchins  
87 Warren Clark  
Atty's

## UNITED STATES PATENT OFFICE.

THOMAS WILLIAM STAINER HUTCHINS, OF DAVENHAM, ENGLAND.

## ELECTRODEPOSITION OF METALS.

Application filed February 5, 1923. Serial No. 617,108.

*To all whom it may concern:*

Be it known that I, THOMAS WILLIAM STAINER HUTCHINS, a subject of the King of Great Britain and Ireland, and resident 5 of Davenham, in the county of Chester, England, have invented certain new and useful Improvements Relating to the Electrodeposition of Metals, of which the following is a specification.

10 In the process of electrolytically depositing metals such as iron, nickel and cobalt, considerable difficulty has been experienced owing to the deposited metal not being homogeneous but exhibiting various faults and 15 being pitted with what are commonly termed hydrogen craters.

It is generally held that hydrogen bubbles result from the decomposition of the water content of the electrolyte and attach 20 themselves to the cathode as points upon which metal is prevented from depositing and numerous attempts have been made to obviate the difficulty either in the direction of preventing the decomposition of the wa- 25 ter content of the electrolyte and therefore the formation of the hydrogen bubbles or in the direction of removing the hydrogen bubbles from the cathode as soon as they are formed.

30 By investigation and experiment, I have found that when solid particles (for instance of carbon) of a nature which would form a couple with the metal deposited are present in the electrolyte, such particles or some 35 of them become attached to the deposited metal and at the point of contact a hydrogen crater or point is formed even though the electrolyte be neutral to methyl orange.

My invention comprises the provision of 40 means which will ensure that the electrolyte round the cathode shall be completely freed from solid foreign matter in suspension of a nature which would form a couple with the metal deposited.

45 My invention further comprises the provision of one or more recuperators containing portions of a similar metal (and/or basic compound or compounds of the same), to that being deposited through which the 50 electrolyte is circulated from and to the electrolyzer, the said recuperators retaining the electrolyte out of contact with the atmosphere so that by the solution of the metal and/or basic compound or compounds of 55 the same to replace at least in part, the metal

deposited at the cathode, the electrolyte is rendered neutral.

In the application of my invention to the electrolytic deposition of iron, the electrolyzer is arranged in series with one or more 60 recuperators containing scrap or other iron and exposing a considerable surface to the action of the electrolyte. The recuperators are sealed against the entry of air and the cross section of such recuperators in proportion to the flow of electrolyte is limited so as to ensure a sufficient scrubbing or washing action on the surface of the scrap metal in such recuperators as to cause the removal therefrom of the impurities in such 70 metal which are insoluble in the electrolyte. The accumulation of such impurities upon the surface of the metal reduces the rate of recuperation of the electrolyte and increases the difficulty of maintaining the latter neu- 75 tral. Further, the area of the electrolyte exposed to the atmosphere is limited in proportion to the area of scrap metal exposed to the electrolyte. The combination of these factors assures the dissolving of the metal 80 by the electrolyte sufficient to replace (either entirely from the scrap iron within the recuperators, or partly therefrom and partly from the anode) the metal deposited at the cathode and to neutralize the action of the 85 atmosphere upon the portion of the electrolyte exposed thereto so restoring the electrolyte to a neutral condition which is of considerable importance in ensuring the de- 90 position of a homogeneous mass.

The electrolyte passing from the recuperators into the electrolyzer is passed through one or more filters which ensure that the liquid delivered therethrough is entirely free from solid matter in suspension of a 95 nature which would form a couple with the metal deposited. If desired, more than one filter may be used, one of which may extract the heavier matter or sludge in a manner similar to that heretofore proposed in connection with electrolytic deposition processes. The final filter or the one which ensures the complete removal of the most minute particles may consist of felt, or earthenware, either alone or in conjunction with a cen- 100 trifugal form of mechanical separator of the hydro-extractor type.

The anode itself is separated from the cathode by means of a diaphragm or filter to prevent any disintegrated solid matter 110

of a nature which would form a couple with the metal deposited passing from the anode into the electrolyte around the cathode. The anode may be made of a 5 metal which is insoluble in the electrolyte and a similar metal to that being deposited (which may be in the form of turnings, filings or like small grade parts) be packed between such anode and the filter or dia- 10 phragm. The use of an insoluble anode in the manner described may considerably cheapen the process.

The electrolyzer may be provided with a readily removable cover for convenience 15 of access to the cathode and the latter may be rotated to ensure evenness of the deposit.

The rate of flow of electrolyte to the electrolyzer should preferably be such that 20 the overflow from the latter (which passes to the recuperator or recuperators) shall be neutral to methyl orange. The solution I prefer to employ as electrolyte preferably consists of:—150 grammes ferrous sulphate— $\text{FeSO}_4(7 \text{ H}_2\text{O})$ , 100 grammes sodium sulphate— $\text{Na}_2\text{SO}_4(10 \text{ H}_2\text{O})$  per litre of water. This may be maintained at a temperature of  $75^\circ$  centigrade during the process.

30 By the process and means aforesaid, I am enabled to deposit homogeneous metal free from pittings or hydrogen craters, the process being simple and requiring only unskilled or semi-skilled labour for its supervision and control. No objectionable fumes or vapours are given off at the electrolyzer and the use of alkalis for neutralizing the electrolyte is obviated. The process is therefore economical and simple and the 35 raw material thereof cheap.

It is understood that whilst the description deals more especially with the deposition of iron, a similar process modified to suit the special conditions serves for the 45 deposition of nickel and/or such other metals as contain amongst their impurities matters which are insoluble in the electrolyte and are of a nature which would form a couple with the metal being deposited.

50 Referring to the accompanying explanatory drawings which illustrate in diagram form, an electrolyzer plant for the deposition of iron, constructed and arranged in one convenient form in accordance with my invention, Figure 1 being a general view of the plant and Figure 2 a cross section of the electrolyzer, the deposition of the metal takes place in the vessel  $\alpha$  in which is mounted a trough-like element  $\beta$  which 55 constitutes the anode and a rotating cylindrical element  $c$  constituting the cathode. The latter in the illustration is disposed horizontally and rotated by a belt pulley  $d$  but it may be disposed vertically. Between 60 the cathode and the anode is arranged a

filter cloth  $e$  as shown in the detail view, Figure 2 which prevents any disintegrated solid matter of a nature which would form a couple with the metal being deposited, from passing into the electrolyte around the 70 cathode.

The vessel  $\alpha$  has a mid-feather  $f$  with an overflow aperture (not shown) therein which allows electrolyte to overflow into the compartment  $g$  whence it flows by the pipe 75  $h$  to the inlet of a pump  $i$ . Electrolyte may flow into the compartment  $g$  along the shaft  $j$  which passes through the mid-feather  $f$ , no packing gland being provided around the shaft, but the amount of electrolyte so 80 flowing will in practice be small.

The electrolyte is circulated by the pump  $i$  through the recuperators  $k l m$  and the filter  $n$  back to the vessel  $\alpha$ . Each of the recuperators is packed with the scrap or 85 other iron and is made of considerable length relatively to its width. A baffle plate  $o$  is provided in each recuperator to prevent the mouth of the liquid pipe being covered by the scrap iron or other material 90 in the recuperator. The vessel  $m$  is steam jacketed for heating purposes.

Each recuperator is sealed by a cover  $p$  against the entry of air and has a sludge 95 cock  $q$  for the withdrawal of solid impurities which accumulate as the iron goes into solution.

The filter  $n$  may be of any suitable construction and arrangement and removes from the electrolyte any solid matter of a 100 nature which would form a couple with the metal being deposited, such as graphite, which may come over from the recuperators.

I claim:—

1. In an apparatus for the electro-deposition of metals, a vessel containing an electrolyte, a cathode and an anode arranged in said vessel, means for circulating the electrolyte, and filtering means arranged immediately adjacent the cathode and isolating the latter from the anode, the filtering means being adapted to completely free the electrolyte around the cathode from all foreign solid impurities of a nature which would become a couple with the metal being deposited.

2. An apparatus as claimed in claim 1 characterized by the provision of a relatively long narrow and air-tight vessel connected with the circulating means and containing metal to be dissolved, said circulating means being adapted to cause the electrolyte to pass through the last mentioned vessel with sufficient velocity to exert a scrubbing action on the metal whereby to remove any impurities in the metal being dissolved from the surface of the same.

3. An apparatus as claimed in claim 1 characterized in that the area of the surface of the electrolyte in contact with the air is

limited to the portion of said electrolyte contained in the vessel whereby, with the assistance of the metal to be dissolved, the electrolyte is maintained in a neutral condition.

4. In an apparatus for electro-deposition of metals, a vessel containing an electrolyte, a cathode and an anode arranged in said vessel, and a filtering diaphragm for filtering the electrolyte, said diaphragm constituting means isolating the cathode from the anode.

5. An apparatus as claimed in claim 4 characterized by the provision of means for circulating the electrolyte, and filtering means arranged in the circulating means, the filtering means being adapted to completely free the electrolyte around the cathode from all foreign solid impurities of a nature which would form a couple with the metal being deposited.

6. An apparatus as claimed in claim 4, characterized by the provision of means for circulating the electrolyte through and externally of the vessel, relatively long narrow and air-tight vessels connected with the circulating means and containing metal to be dissolved, means for passing the electrolyte through the last mentioned vessels with sufficient velocity to exert a scraping action on the metal whereby to remove any impurities in the metal being dissolved from the surface of the same.

7. An apparatus as claimed in claim 4 characterized by the provision of means for circulating the electrolyte through and externally of the vessel, relatively long narrow and air-tight vessels connected with

the circulating means and containing metal to be dissolved, means for passing the electrolyte through the last mentioned vessels with sufficient velocity to exert a scraping action on the metal whereby to remove any impurities in the metal being dissolved from the surface of the same, and filtering means arranged in the circulating means for filtering out the impurities.

8. An apparatus as claimed in claim 4 characterized by the provision of means for circulating the electrolyte, vessels connected with the circulating means and containing metal to be dissolved, said circulating means acting to pass the electrolyte through the last mentioned vessels with sufficient velocity to exert a scraping action on the metal whereby to remove any impurities in the metal being dissolved from the surface of the same, and means rendering the last mentioned vessels air-tight whereby the area of the surface of the electrolyte in contact with the air is limited to the portion of said electrolyte contained in the vessel, and with the assistance of the metal to be dissolved, the electrolyte is maintained in a neutral condition.

9. In an apparatus for electro-deposition of metals, a vessel containing an electrolyte, a cathode and an anode arranged in said vessel filtering means arranged between the cathode and anode, said anode being insoluble in the electrolyte, and a metal similar to that being deposited packed between the anode and filtering means.

In testimony whereof I have signed my name to this specification.

THOMAS WILLIAM STAINER HUTCHINS.